

## UNITED STATES PATENT OFFICE

2,424,552

## FROTH FLOTATION OF NONMETALLIC MINERALS

Julius Bruce Clemmer and Carl Rampacek,  
Tuscaloosa, Ala.No Drawing. Application May 1, 1945,  
Serial No. 591,293

8 Claims. (Cl. 209—166)

(Granted under the act of March 3, 1883, as  
amended April 30, 1928; 370 O. G. 757)

1

The invention described herein may be manufactured and used by or for the Government of the United States for governmental purposes without the payment to us of any royalty thereon in accordance with the provisions of the act of April 30, 1928 (Ch. 460, 45 Stat. L. 467).

This invention relates to an improved process for the concentration of nonmetallic minerals from ores containing them in association with siliceous gangue; more particularly it relates to a froth flotation process employing anionic collecting agents to effect flotation of activated siliceous gangue constituents from nonmetallic ores. The term "nonmetallic" is used herein to designate those minerals which are used commercially for purposes other than as a source of metal which they contain. Among the so designated nonmetallic minerals are included phosphates, calcite, barite, strontianite, and witherite. The present invention herein described relates to the froth flotation of activated siliceous gangue constituents from all five of these minerals.

An object of the invention is to provide an improved process for the concentration of nonmetallic minerals in pulps containing them in the presence of siliceous gangue. A further object is to provide a flotation process which will have greater selectivity in separating siliceous materials from nonmetallic ores and thereby effect greater operating economies. A still further object is to provide a froth flotation process for siliceous gangue materials wherein inexpensive anionic collecting agents are employed to float the siliceous gangue. Other objects, purposes, and advantages of the invention will hereinafter more fully appear or will be understood from the detailed description of its practice.

We are aware that various froth flotation methods have been proposed for the concentration of nonmetallic ores for the purpose of rejecting siliceous gangue constituents and recovering an enriched product of the economic nonmetallic minerals. A conventional flotation method well known to the art is to float the economic nonmetallic minerals from the siliceous gangue materials employing oleic acid, sodium oleate, or similar anionic collecting agents in conjunction with various addition agents in acid, neutral, or moderately alkaline pulps to facilitate flotation of the desired nonmetallic mineral from the retarded silica. The technical and patent literature abounds with examples of practice of the methods for the flotation of such nonmetallic minerals as rock phosphate, calcite, barite, and fluorspar from quartz, feldspar, and other siliceous gangue materials. Among others, for example, Crago describes a method for the anionic flotation of

2

fluorspar or phosphate rock from siliceous gangue in U. S. Patent 2,105,807. Tartaron in U. S. Patent 2,105,826 makes use of the short chain fatty acid collectors and various metal salts to effect flotation of phosphate rock, calcite, barite, or fluorspar from siliceous gangue in substantially neutral or acid pulps. Rose and MacDonald in U. S. Patent 2,040,187 describes the flotation of carbonates, sulfates, fluorides, tungstates, and oxides from each other and from siliceous gangue by the use of fatty acid collecting agents in conjunction with various metallic salts in the presence of a metaphosphate or similar addition agent. These and numerous other investigators have made use of various anionic collectors in conjunction with a variety of inorganic and organic addition agents to enable flotation of non-sulfide metallic and nonmetallic minerals from each other and from siliceous gangue in particular.

An alternative method for concentrating nonmetallic minerals by flotation is to reverse the customary separation and float the siliceous gangue constituents from the nonmetallic carbonate, sulfate, or phosphate minerals employing cationic collecting agents such as laurylamine hydrochloride, cetyl trimethyl ammonium bromide, or similar compounds which ionize in the aqueous pulps to yield a large active cation. Collectors of the cationic type have been used and found advantageous for the flotation of siliceous gangue from many nonmetallic ores. Among others, for example, Tartaron describes a method for the cationic flotation of silica from phosphates, calcite, barite, and fluorspar in U. S. Patent 2,222,728 and Breerwood and Williams in U. S. Patent 2,161,010 made use of cationic collectors for floating siliceous constituents from cement rock. Despite their widespread adoption for the flotation of silica and silicates from non-sulfide and nonmetallic ores and mineral products, cationic collectors have many limitations. They are more expensive than collectors of the anionic type, and, moreover, they are not particularly selective. Cationic collectors are ineffective silica collectors in the presence of slime and desliming of the ore pulp is generally necessary before satisfactory flotation separation can be achieved.

As a result of extended research and experimentation, we have discovered a method of concentrating nonmetallic ores by froth flotation wherein anionic collecting agents are employed to float activated siliceous gangue constituents from caustic alkaline ore pulps with a pH of at least 10 while retarding flotation of the economic nonmetallic mineral with a soluble inorganic metaphosphate or polyphosphate. A moderate quan-

tity of a meta- or poly-phosphate in a strongly caustic alkaline pulp of the non-metallic ore effectively retards flotation of such nonmetallic minerals as calcium phosphate in phosphate rock, calcite in cement rock, and barite, strontianite, or witherite without adversely affecting anionic flotation of the activated silica.

In a co-pending application, assigned to the same assignee as the present application, by Julius Bruce Clemmer and Ballard H. Clemmons, Serial No. 473,162, filed January 22, 1943, is described a process for beneficiating iron ores and products from the milling of iron ores containing calcareous and/or siliceous gangue materials wherein anionic collecting agents are employed to float the activated siliceous constituents from caustic alkaline iron ore pulps with a pH of at least 10 while retarding flotation of the iron oxides with a metaphosphate or polyphosphate. Choice of the quantity of phosphate and collector employed in flotation of the calcareous iron ores enables flotation of the calcareous constituents with the activated silica or retardation of the calcareous materials with the iron oxides. The present application is an outgrowth of the aforementioned invention with particular reference to the concentration of nonmetallic ores and mineral products.

A caustic alkaline pulp with a pH at least as high as 10, and preferably in the pH range 10 to 12, is preferable in our method of flotation to facilitate effective retardation of the economic nonmetallic minerals by the meta- or poly-phosphate depressants during flotation of the silica. We prefer to employ caustic alkalies, such as sodium or potassium hydroxides, or their equivalents, to establish the desired pH for flotation. Moderate quantities of other alkaline reagents, such as sodium sulfide, sodium carbonate, and sodium silicate, may be used in conjunction with the caustic alkalies if desired. A combination of hydrated lime and soda ash has been successfully employed in the flotation of many nonmetallic ores and served the dual purpose of activating the siliceous materials to anionic flotation and establishing the desired caustic alkalinity for flotation by formation of caustic soda within the pulp. The optimum pH for anionic flotation of the activated siliceous constituents and retardation of the desired nonmetallic mineral to be recovered varies slightly for different ores but generally falls within the range 10 to 12, and the proper pH for any particular case is best determined by experimentation. Poor flotation of the silica and incomplete retardation of the nonmetallic invariably results if the pH of the pulp is much less than 10; a pulp pH greater than 12 is not particularly objectionable in our method of flotation, but the froth is inclined to be voluminous and flotation of the silica is sluggish. We, therefore, prefer in our flotation method to keep the pH in the range of 10 to 12.

It is essential in the practice of this invention that the siliceous gangue constituents in the non-metallic ore be activated and rendered floatable. The siliceous gangue materials in certain non-metallic ores, such as the cement rocks containing quartz associated with calcite or limestone, are naturally activated to soap flotation, presumably due to soluble calcium salts in the ore. Other nonmetallic ores, however, seldom contain naturally activated siliceous materials and the successful operation of our process requires that the silica in such ores be activated for anionic flotation. Extended research of a variety

of nonmetallic ores demonstrated that our method of flotation lends itself readily to the use of silica activating agents. Many alkaline-earth and heavy metal salts exhibit the property of activating quartz and various silicate minerals to soap flotation when a proper quantity is employed at an optimum pH. We have found that conditioning of the caustic alkaline ore pulp with a moderate quantity of an activator selected from the group consisting of soluble calcium, magnesium, barium, strontium, and lead salts suffices to activate the siliceous gangue constituents in many nonmetallic ores to anionic flotation by the higher fatty acids, resin acids, or their derived soaps, without adversely affecting retardation of the economic nonmetallic mineral by the phosphate depressants. The effectiveness of the metal salt activating agents differs for different ores and the proper quantity for any particular case is best determined by experimentation. A proper quantity of metal salt activating agent, collector, and phosphate depressant in a caustic alkaline pulp with a pH of 10 to 12 enables rapid and substantially complete flotation of silica from calcium phosphate, calcite, barite, strontianite, or witherite.

We may also employ hydrated lime as the silica activating agent in the practice of our invention, and from the standpoint of cost, hydrated lime is particularly attractive. Grinding or blunging the ore with sufficient hydrated lime to establish a pulp pH of about 11 effects substantially complete activation of the silica. The usual quantity of hydrated lime required to activate the silica varies from 1 to 4 pounds per ton of ore, but some ores containing acidic salts may require 8 pounds or more of lime per ton. Excessive quantities of dissolved hydrated lime in the conditioned pulp should be removed before flotation as they increase collector and phosphate requirements. Although we have achieved by the practice of our invention good flotation of silica from nonmetallic ore pulps containing as much as 100 parts per million of hydrated lime in solution, equivalent in our tests to about 0.8 pound of hydrated lime per ton of solids, we prefer that the pulp for flotation be substantially free of dissolved hydrated lime. The lime salts in the conditioned pulp may be removed by settling and washing the pulp with fresh water, or by addition of sufficient soda ash to the pulp to precipitate the dissolved lime as insoluble calcium carbonate. The combination of hydrated lime and soda ash was particularly advantageous on many ores; conditioning the ore pulp with hydrated lime to give a pH of about 11 sufficed for activation of the silica and subsequent addition of soda ash to precipitate the dissolved hydrated lime remaining in solution gave a pulp of the desired caustic alkalinity for flotation. Additional caustic soda may be added to the pulp if desired. Should an excess of hydrated lime be inadvertently added to the pulp to activate the silica, as evidenced by a pH of about 12.3 which is the pH of a saturated solution of hydrated lime, the excess is best removed by settling and washing the pulp one or more times with fresh water to reduce the pH to about 11, whereupon soda ash may be added to precipitate the dissolved lime remaining in the pulp before proceeding with flotation. If desired, however, the washing may be carried further to give a final pulp for flotation practically free of dissolved hydrated lime and having a pH of 9 to 10. Subsequent addition of a caustic alkali to the lime conditioned and washed pulp to estab-

lish the desired pH for flotation together with a higher fatty acid, resin acid, or soap collecting agent in conjunction with a metaphosphate or polyphosphate enables flotation of the calcium-activated silica and retardation of the economic nonmetallic mineral.

The use of a soft water free of lime or magnesium salts is not obligatory in the practice of this invention. A water moderately hard with lime salts, for example, is permissible and, in fact, has been found advantageous as the lime salts aid in the activation of the siliceous materials.

The anionic collecting agents which we have found suitable for flotation of activated siliceous gangue materials from nonmetallic ores include oleic acid, red oil (crude oleic acid), crude and purified sodium oleate, fish oil fatty acids, fish oil soaps, and various crude or purified talols and sulfate soaps recovered from sulfate paper mill black liquors. The talols, which are mixtures of fatty and resin acids, are relatively inexpensive and are particularly attractive collectors on many nonmetallic ores.

The various phosphates which we have employed and found suitable for retarding flotation of nonmetallic minerals in the practice of our invention include sodium metaphosphate, sodium hexametaphosphate, and sodium tetraphosphate. The potassium salts may also be employed if desired, but they are more expensive than the sodium salts. The alkali-metal salts of the ortho- and pyro-phosphates lack the specific depressing properties of the meta- and poly-phosphates, but have been employed as auxiliary reagents in the practice of our invention to aid pulp dispersion and improve the flotation separation.

While we have achieved satisfactory flotation of activated silica from nonmetallic ore pulps containing substantial quantities of slime by the practice of our invention, we prefer that the flotation pulp be deslimed. Desliming of the pulp should be practiced whenever permissible as subsequent flotation of the activated silica is more rapid and complete, and less reagents are required in flotation.

The proportions of the various reagents employed in the practice of our flotation method are subject to considerable variation, and the optimum quantities are best determined by experimentation for any particular case. Purity of the separated products is a reliable guide for reagent adjustment. An excess of collecting agent promotes flotation of a portion of the economic nonmetallic mineral with the activated siliceous gangue, whereas a deficiency of collector results in incomplete flotation of the silica. Conversely, an excess of metaphosphate or polyphosphate results in retardation of a portion of the siliceous gangue, whereas a deficiency permits flotation of the economic nonmetallic mineral with the silica. Control of the collector and phosphate depressant is not critical, however, and reasonable variations in the quantities employed is permissible without adversely affecting the separation.

Conventional flotation terminology designates the floated product from roughing and cleaning operations as concentrates, and the pulp residues as tailings and middlings, respectively. This terminology is in keeping with the general practice of floating the valuable mineral from the worthless gangue. When the separation is reversed and the gangue is floated from the economic mineral, the terminology may become confused. To avoid possible confusion in describing the results of our flotation tests, we shall here-

inafter designate the enriched pulps of the economic nonmetallic mineral from the roughing and cleaning steps as "concentrates, rougher" and "concentrates, cleaner," respectively. The floated silica products from the roughing and cleaning steps will be designated as "rougher froth" and "silica rejects," respectively. In describing the results of our flotation tests we shall for simplicity hereinafter consider and report the enriched pulps from the cleaning steps (middlings) as finished concentrates. It will be readily apparent to those skilled in the art that the middlings may be retreated by conventional methods to yield an even higher grade concentrate without departing from the spirit of the invention.

The invention will be further illustrated, but is not intended to be limited by the following examples of practice:

#### Example I

A sample of deslimed phosphate feed was obtained from an operating washer near Brewster, Florida, in the land-pebble phosphate district. The sample consisted mainly of so-called bone phosphate of lime (tricalcium phosphate) associated with quartz and some indurated clay. A head analysis gave 59.3 percent  $\text{Ca}_3(\text{PO}_4)_2$ , hereinafter referred to as B. P. L. for convenience, and 19.6 percent  $\text{SiO}_2$ . The sample as received was substantially finer than 20 mesh and was used for the following flotation procedures.

A 250-gram portion of the phosphate sample was wet ground to pass 65 mesh in a laboratory pebble mill. The ground charge was diluted to a volume of 2.5 liters with additional tap water to give a pulp containing about 10 percent solids. The pulp was dispersed using caustic soda and sodium hexametaphosphate equivalent to 1.0 and 0.5 pound per ton of ore, respectively. The dispersed pulp was fractionated by sedimentation and decantation to remove the bulk of the slime finer than 20 microns. The deslimed granular portion of the ore was repulped with additional tap water and transferred to a small mechanical agitation flotation cell of standard design. Additional tap water was added to the cell to give a pulp for flotation containing about 20 percent solids. Flotation of the siliceous gangue from the calcium phosphate was achieved by employing the following reagent charge expressed in conventional pounds per ton of ore:

| 55 | Reagent                        | Conditioner |       | Rougher | Scavenger | Cleaner |       |
|----|--------------------------------|-------------|-------|---------|-----------|---------|-------|
|    |                                | No. 1       | No. 2 |         |           | No. 1   | No. 2 |
|    | Caustic soda.....              | 1.5         | ..... | .....   | .....     | 0.5     | 0.5   |
|    | Sodium hexameta-phosphate..... | 1.0         | ..... | .....   | 0.4       | 0.04    | 0.2   |
| 60 | Talol.....                     | .....       | 0.6   | .....   | 0.4       | 0.2     | ..... |
|    | Calcium chloride.....          | .....       | 1.0   | .....   | .....     | 0.2     | ..... |
|    | Time, min.....                 | 2.5         | 2.5   | 3.0     | 3.0       | 3.0     | 2.5   |
|    | Pulp pH.....                   | 10.9        | 10.6  | 10.4    | 10.0      | 10.2    | 10.2  |

The substantially deslimed pulp was first conditioned with the caustic soda (commercial lye) and sodium hexametaphosphate to retard the calcium phosphate and establish the desired caustic alkalinity for activation and flotation of the silica. The pulp was then conditioned with calcium chloride and talol to activate and float the silica. Air was then allowed to enter the cell and resulted in immediate formation of a compact, heavily mineralized froth of the siliceous gangue materials. The froth was collected for 3.0 minutes whereupon flotation of the

calcium-activated silica was substantially complete. Additional talol was then added to the pulp and a scavenger product was obtained by collecting the resulting froth for 3.0 minutes. The rougher and scavenger froths were combined and cleaned twice by refloating in the same cell using tap water for dilution and the quantities of reagents as indicated. The final silica rejects, the combined phosphate concentrates from the cleaning steps (middlings), the rougher phosphate concentrate (tailing), and the untreated slime were dried, weighed, and analyzed. The results of the test are as follows.

| Product                        | Weight, per cent | Assay, per cent |                  | Dist., per cent |                  |
|--------------------------------|------------------|-----------------|------------------|-----------------|------------------|
|                                |                  | B. P. L.        | SiO <sub>2</sub> | B. P. L.        | SiO <sub>2</sub> |
| <b>Phosphate Concentrates:</b> |                  |                 |                  |                 |                  |
| Rougher.....                   | 63.2             | 67.8            | 8.2              | 72.1            | 26.9             |
| Cleaner.....                   | 13.2             | 64.5            | 12.0             | 14.3            | 8.3              |
| Slime (untreated).....         | 11.0             | 64.0            | 11.9             | 11.9            | 6.8              |
| Composite.....                 | 87.4             | 66.8            | 9.2              | 98.3            | 42.0             |
| Silica Rejects.....            | 12.6             | 7.9             | 88.0             | 1.7             | 58.0             |
| Composite Feed                 | 100.0            | 59.4            | 19.1             | 100.0           | 100.0            |

The flotation silica rejects, which accounted for 12.6 percent of the weight of the feed, contained 58.0 percent of the silica and only 1.7 percent of the B. P. L. The untreated slime and the cleaner phosphate concentrates were sufficiently free of silica to be considered finished grade. The composited phosphate concentrates accounted for a recovery of 98.3 percent of the phosphate in the sample and analyzed 66.8 percent B. P. L and 9.2 percent SiO<sub>2</sub>.

#### Example II

Another 250-gram portion of the phosphate sample was wet ground in a laboratory pebble mill to pass 65 mesh in the presence of hydrated lime equivalent to 12.0 pounds per ton of ore. The ground charge, which had a pH of 11.2 due to presence of hydrated lime, was flocculated and settled readily. The clear, supernatant 40 grind water was carefully decanted from the settled material to avoid loss of solids. The settled material was repulped with 5 liters of fresh tap water and again allowed to stand until the solids had settled. The clear, supernatant water 45 was decanted from the solids and the washing operation was again repeated. The twice-washed pulp had a pH of 9.8 and was substantially free of hydrated lime. The washed pulp was then transferred to a laboratory flotation 50 cell and enough tap water was added to give a pulp for flotation containing about 20 percent solids. Flotation of the lime-activated silica from the calcium phosphate was effected by the following reagents expressed in conventional 55 pounds per ton of ore:

| Reagent                            | Conditioner |       | Rough-<br>er | Scav-<br>enger | Cleaner |       |  |  |
|------------------------------------|-------------|-------|--------------|----------------|---------|-------|--|--|
|                                    | No. 1       | No. 2 |              |                | No. 1   | No. 2 |  |  |
|                                    |             |       |              |                |         |       |  |  |
| Caustic soda.....                  | 1.2         | —     | —            | —              | 0.4     | —     |  |  |
| Sodium hexameta-<br>phosphate..... | 1.5         | —     | —            | —              | 0.04    | —     |  |  |
| Talol.....                         | —           | 0.6   | —            | —              | 0.4     | 0.2   |  |  |
| Lead nitrate.....                  | —           | —     | —            | —              | 0.4     | —     |  |  |
| Time, min.....                     | 2.5         | 2.5   | 5.0          | 3.0            | 5.0     | 5.0   |  |  |
| Pulp pH.....                       | 11.2        | 10.9  | 10.6         | 10.0           | 10.0    | 10.0  |  |  |

The slime-bearing pulp was conditioned with caustic soda (commercial lye) and sodium hexametaphosphate. Talol was then added and 75

the pulp again briefly conditioned. Air was admitted to the flotation cell and the rougher froth was removed. Additional talol and a small quantity of lead nitrate were added to the pulp to activate and float the remaining silica in a scavenger froth. The rougher and scavenger froths were combined and cleaned twice by refloating in the same cell. Tap water was used for dilution together with the quantities of reagents as indicated. The rougher and composited cleaner phosphate concentrates, and the final silica rejects were dried, weighed, and analyzed. The results of the test are as follows:

| Product                        | Weight, per cent | Assay, per cent |                  | Dist., per cent |                  |
|--------------------------------|------------------|-----------------|------------------|-----------------|------------------|
|                                |                  | B. P. L.        | SiO <sub>2</sub> | B. P. L.        | SiO <sub>2</sub> |
| <b>Phosphate Concentrates:</b> |                  |                 |                  |                 |                  |
| Rougher.....                   | 65.9             | 66.3            | 10.0             | 73.9            | 34.0             |
| Cleaner.....                   | 11.9             | 65.0            | 11.4             | 13.1            | 7.0              |
| Slime (untreated).....         | 10.9             | 64.2            | 11.8             | 11.8            | 6.6              |
| Composite.....                 | 88.7             | 65.9            | 10.4             | 98.8            | 47.6             |
| Silica Rejects.....            | 11.3             | 6.0             | 90.0             | 1.2             | 52.4             |
| Composite Feed                 | 100.0            | 59.1            | 19.4             | 100.0           | 100.0            |

Anionic flotation of the lime-activated silica rejected 81.5 percent of the silica in the feed with a loss of only 8.3 percent of the B. P. L. Flotation of the silica from the slime-bearing pulp was readily achieved. It is therefore apparent that our method of flotation is applicable to slime-bearing as well as deslimed pulps.

#### Example III

Another portion of the Florida phosphate sample was ground to pass 65 mesh, deslimed, and floated by the procedure described in Example I, but in this instance lead nitrate was employed to activate the silica to anionic flotation. The reagent charge employed in the test was as follows:

| Reagent                            | Conditioner |       | Rough-<br>er | Scav-<br>enger | Cleaner |       |
|------------------------------------|-------------|-------|--------------|----------------|---------|-------|
|                                    | No. 1       | No. 2 |              |                | No. 1   | No. 2 |
| Caustic soda.....                  | 2.0         | —     | —            | —              | 0.5     | 0.5   |
| Sodium hexameta-<br>phosphate..... | 0.5         | —     | —            | —              | 0.2     | —     |
| Talol.....                         | —           | 1.0   | —            | —              | 0.4     | —     |
| Lead nitrate.....                  | —           | 1.0   | —            | —              | 0.4     | —     |
| Time, min.....                     | 2.5         | 2.5   | 3.0          | 3.0            | 2.5     | 2.5   |
| Pulp pH.....                       | 11.2        | 11.0  | 10.1         | 9.5            | 10.9    | 10.7  |

The results of the test are as follows:

| Product                        | Weight, per cent | Assay, per cent |                  | Dist., per cent |                  |
|--------------------------------|------------------|-----------------|------------------|-----------------|------------------|
|                                |                  | B. P. L.        | SiO <sub>2</sub> | B. P. L.        | SiO <sub>2</sub> |
|                                |                  |                 |                  |                 |                  |
| <b>Phosphate Concentrates:</b> |                  |                 |                  |                 |                  |
| Rougher.....                   | 65.9             | 66.3            | 10.0             | 73.9            | 34.0             |
| Cleaner.....                   | 11.9             | 65.0            | 11.4             | 13.1            | 7.0              |
| Slime (untreated).....         | 10.9             | 64.2            | 11.8             | 11.8            | 6.6              |
| Composite.....                 | 88.7             | 65.9            | 10.4             | 98.8            | 47.6             |
| Silica Rejects.....            | 11.3             | 6.0             | 90.0             | 1.2             | 52.4             |
| Composite Feed                 | 100.0            | 59.1            | 19.4             | 100.0           | 100.0            |

The results of the previously recorded flotation tests are typical of those we have obtained on samples of deslimed feed from several washers operating in the Florida phosphate district. Flotation of total or deslimed charges of the washer feeds ground in a pebble mill, iron ball-mill, or iron rod-mill to pass 65, 100, or 200 mesh gave results similar to those indicated. A moderate quantity of a metaphosphate or polyphosphate,

such as sodium metaphosphate, sodium hexametaphosphate, or sodium tetraphosphate, in a caustic alkaline pulp having a pH of at least 10, and preferably 11 to 12, adequately retarded the calcium phosphate during flotation of the activated silica. Hydrated lime and various soluble alkaline-earth and heavy-metal salts, such as calcium chloride, magnesium sulfate, barium chloride, strontium nitrate, or lead nitrate, were employed and found suitable for activating the quartz and granular silicate minerals to anionic flotation. 15 Tallol, sulfate soap, oleic acid, sodium oleate, fish oil soap, fish oil fatty acids, and similar anionic collecting agents were employed in various tests for flotation of the activated silica and gave good results. The proper quantity of caustic alkali, phosphate depressant, activating agent, and collector differs slightly for different ores and the optimum quantities are best determined by trial for each particular case.

*Example IV*

A synthetic cement rock was prepared by mixing approximately equal quantities of calcite and quartz. The mixture was ground to pass 65 mesh in a laboratory pebble mill and transferred to a laboratory mechanical flotation cell. Tap water was added to the cell to give a pulp containing about 25 percent solids. Flotation of the quartz from the calcite was effected by the following reagents expressed in conventional pounds per ton of flotation feed:

| Reagent                  | Conditioner |       | Rougher |
|--------------------------|-------------|-------|---------|
|                          | No. 1       | No. 2 |         |
| Caustic soda             | 1.0         |       |         |
| Sodium hexametaphosphate | 1.0         | 0.5   |         |
| Calcium Chloride         |             | 1.0   |         |
| Sodium oleate            |             | 0.8   |         |
| Oleic acid               | 2.5         | 1.5   | 2.5     |
| Time, min.               | 11.2        | 11.2  | 10.7    |
| Pulp pH                  |             |       |         |

The pulp was first conditioned with caustic soda and sodium hexametaphosphate to retard the calcite and establish the desired caustic alkaline pulp for activation and flotation of the quartz. The pulp was then conditioned with calcium chloride, sodium oleate, and oleic acid to activate and float the quartz. Air was then admitted to the cell and resulted in immediate formation of a silica rougher froth which was sufficiently free of calcite to be rejected without cleaning. The results of the flotation test follow:

| Product                      | Weight, per cent | Assay, per cent   |                  | Dist., per cent   |                  |
|------------------------------|------------------|-------------------|------------------|-------------------|------------------|
|                              |                  | CaCO <sub>3</sub> | SiO <sub>2</sub> | CaCO <sub>3</sub> | SiO <sub>2</sub> |
|                              |                  |                   |                  |                   |                  |
| Calcite concentrate, rougher | 51.9             | 89.3              | 10.7             | 93.0              | 11.1             |
| Silica rougher froth         | 48.1             | 7.2               | 92.8             | 7.0               | 88.9             |
| Composite Feed               | 100.0            | 50.2              | 49.8             | 100.0             | 100.0            |

Rougher flotation of the quartz rejected 88.9 percent of the silica with a loss of only 7.0 percent of the calcium carbonate.

*Example V*

Another portion of the synthetic cement rock was ground to pass 65 mesh and floated by the procedure described in Example IV, but in this instance lead nitrate and tallol were employed to activate and float the quartz from the calcite. The silica rougher froth was cleaned twice by 75 insure complete activation of quartz, chert, feld-

refloating in the same cell using tap water for dilution. The reagent charge employed in the test was as follows:

| 5  | Reagent                  | Conditioner |       | Rougher | Cleaner |       |
|----|--------------------------|-------------|-------|---------|---------|-------|
|    |                          | No. 1       | No. 2 |         | No. 1   | No. 2 |
| 10 | Caustic soda             | 0.7         |       |         | 0.4     | 0.4   |
|    | Sodium hexametaphosphate | 1.0         |       |         | 0.05    | 0.10  |
|    | Lead nitrate             | 1.0         |       |         |         |       |
|    | Tallol                   |             |       | 1.0     |         |       |
|    | Time, min.               | 2.5         | 2.5   | 3.0     | 2.5     | 2.0   |
|    | Pulp pH                  | 11.2        | 11.2  | 11.0    | 10.8    | 10.7  |

The results of the test follow:

| 20 | Product             | Weight, per cent | Assay, per cent   |                  | Dist., per cent   |                  |
|----|---------------------|------------------|-------------------|------------------|-------------------|------------------|
|    |                     |                  | CaCO <sub>3</sub> | SiO <sub>2</sub> | CaCO <sub>3</sub> | SiO <sub>2</sub> |
|    | Calcite concentrate | 35.8             | 99.3              | 0.7              | 70.3              | 0.5              |
|    | Middlings           | 33.2             | 39.8              | 60.2             | 26.1              | 40.5             |
|    | Silica Rejects      | 31.0             | 5.9               | 94.1             | 3.6               | 59.0             |
|    | Composite Feed      | 100.0            | 50.6              | 49.4             | 100.0             | 100.0            |

25 The calcite concentrate (rougher tailing) and silica rejects (cleaner froth) from the test were of acceptable grade, but the middlings would require retreatment to yield final concentrates and tailings.

*Example VI*

35 Another synthetic cement rock was prepared by mixing approximately 7 parts of calcite and 3 parts of quartz. The mixture was wet ground in a pebble mill to pass 65 mesh. Qualitative tests on the grind water showed presence of calcium salts. The ground pulp was transferred to a flotation cell and diluted with enough tap water to give a pulp containing about 25 percent solids. The quartz was floated from the calcite by the following reagent charge:

| 45 | Reagent                  | Conditioner |       | Rougher | Scavenger |
|----|--------------------------|-------------|-------|---------|-----------|
|    |                          | No. 1       | No. 2 |         |           |
|    | Caustic soda             | 1.0         |       |         |           |
|    | Sodium hexametaphosphate | 1.0         |       |         |           |
|    | Sodium oleate            |             |       | 1.0     |           |
|    | Oleic acid               |             |       | 0.4     | 0.4       |
| 40 | Time, min.               | 2.5         | 2.5   | 2.5     | 2.5       |
|    | Pulp pH                  | 11.2        | 11.2  | 11.1    | 11.0      |

55 The rougher and scavenger froths in the tests were sufficiently free of calcite to be rejected without cleaning. Analysis of the calcite concentrate and the combined rougher and scavenger silica froths gave the following results:

| 60 | Product             | Weight, per cent | Assay, per cent   |                  | Dist., per cent   |                  |
|----|---------------------|------------------|-------------------|------------------|-------------------|------------------|
|    |                     |                  | CaCO <sub>3</sub> | SiO <sub>2</sub> | CaCO <sub>3</sub> | SiO <sub>2</sub> |
|    |                     |                  |                   |                  |                   |                  |
|    | Calcite Concentrate | 76.1             | 90.3              | 9.7              | 98.1              | 24.7             |
|    | Silica Rejects      | 23.9             | 5.7               | 94.3             | 1.9               | 75.3             |
| 65 | Composite Feed      | 100.0            | 70.1              | 29.9             | 100.0             | 100.0            |

In the recorded test, good flotation of quartz from calcite was achieved without use of supplementary addition agents to activate the quartz. The calcium salts released in the pulp upon grinding the mixture to flotation size was enough to activate the quartz to soap flotation. In the practice of our invention, however, we may use a soluble alkaline-earth or heavy-metal salt to insure complete activation of quartz, chert, feld-

11

spar, or other silicate gangue minerals that we wish to reject by anionic flotation. A moderate quantity of a calcium or lead salt, for example, in conjunction with an anionic collecting agent permits more complete flotation of the siliceous gangue constituents from the retarded economic non-metallic mineral to yield higher grade concentrates.

*Example VII*

In another test on the aforementioned synthetic cement rock wherein lead nitrate equivalent to 1.0 pound per ton of flotation feed was employed to activate the quartz, the calcite concentrates assayed 98.9 percent  $\text{CaCO}_3$  and 1.1 percent  $\text{SiO}_2$ , and the silica rejects assayed 21.2 percent  $\text{CaCO}_3$  and 78.8 percent  $\text{SiO}_2$ .

*Example VIII*

In still another test on the synthetic cement rock, hydrated lime equivalent to 12 pounds per ton of flotation feed was added to the grinding operation. The ground pulp was washed with fresh tap water to reject the lime remaining in solution employing the procedure described in Example II. The washed pulp was floated to reject the quartz using 1.0, 0.6, 1.0, and 0.4 pound per ton, respectively, of caustic soda, sodium hexametaphosphate, sodium oleate, and oleate acid. The rougher calcite concentrate assayed 99.0 per cent  $\text{CaCO}_3$  and 1.0 per cent  $\text{SiO}_2$ , and accounted for a recovery of 94.1 percent of the calcium carbonate in the feed. The rougher silica froth assayed 13.0 per cent  $\text{CaCO}_3$  and 87.0 percent  $\text{SiO}_2$ , and contained 97.6 per cent of the silica in the feed.

*Example IX*

A mixture composed of approximately 6 parts of witherite and 4 parts of quartz was ground to pass 65 mesh and subjected to flotation in a manner similar to that described in Example IV. Activation and flotation of the quartz from the witherite was effected by the following reagents expressed in pounds per ton of flotation feed:

| Reagent                  | Conditioner |       |       | Rougher | Scavenger | Cleaner |
|--------------------------|-------------|-------|-------|---------|-----------|---------|
|                          | No. 1       | No. 2 | No. 3 |         |           |         |
| Calcium chloride         | 1.0         |       |       |         |           | 0.4     |
| Caustic soda             |             | 1.0   |       |         |           | 0.04    |
| Sodium hexametaphosphate |             | 1.0   |       |         |           | 0.04    |
| Sodium oleate            |             |       | 1.0   |         |           | 0.10    |
| Oleic acid               |             |       | 0.4   |         |           | 0.10    |
| Time, min.               | 2.5         | 2.5   | 2.5   | 2.5     | 2.5       | 2.5     |
| Pulp pH                  | 11.2        | 11.2  | 11.2  | 10.7    | 10.7      | 10.8    |

The rougher and scavenger silica froths were combined and cleaned once in the same cell using tap water for dilution with caustic soda to maintain alkalinity, sodium hexametaphosphate to retard the witherite, and sodium oleate to insure flotation of the quartz. The results of the test are as follows:

| Product                 | Weight, per cent | Assay, per cent |                | Dist., per cent |                |
|-------------------------|------------------|-----------------|----------------|-----------------|----------------|
|                         |                  | $\text{BaCO}_3$ | $\text{SiO}_2$ | $\text{BaCO}_3$ | $\text{SiO}_2$ |
| Witherite Concentrates: |                  |                 |                |                 |                |
| Rougher                 | 45.1             | 99.0            | 1.0            | 76.5            | 1.1            |
| Cleaner                 |                  | 84.0            | 16.0           | 12.7            | 3.4            |
|                         |                  |                 |                |                 |                |
| Composite               |                  | 53.9            | 96.6           | 3.4             | 89.2           |
|                         |                  | 46.1            | 13.8           | 86.2            | 10.8           |
| Silica Rejects          |                  |                 |                |                 | 4.5            |
|                         |                  |                 |                |                 | 95.5           |
| Composite Feed          |                  | 100.0           | 58.4           | 41.6            | 100.0          |
|                         |                  |                 |                |                 | 100.0          |

12

Anionic flotation of the calcium-activated quartz rejected 95.5 percent of the silica in the feed with a loss of 10.8 percent of the barium carbonate (witherite).

In this test, the calcium chloride used to activate the quartz to anionic flotation was added to the pulp before the alkali and phosphate. While we have found that such practice is permissible on many nonmetallic ores, we generally prefer to add the silica-activating agent to the caustic alkaline and phosphate conditioned pulp. The soluble alkaline-earth or heavy-metal salt to activate the silica may be added before, with, or after the anionic collecting agent without departing from the spirit of our invention.

*Example X*

A mixture composed of approximately 6 parts of strontianite and 4 parts of quartz was ground to pass 65 mesh and subjected to flotation in a manner similar to that described in Example IV. Activation and flotation of the quartz from the strontianite was achieved by the following reagents expressed in conventional pounds per ton of flotation feed:

| Reagent                  | Conditioner |       | Rougher | Cleaner |
|--------------------------|-------------|-------|---------|---------|
|                          | No. 1       | No. 2 |         |         |
| Caustic soda             | 1.0         |       |         |         |
| Sodium hexametaphosphate | 0.5         |       |         |         |
| Calcium chloride         | 1.0         |       |         |         |
| Sodium oleate            |             | 2.0   |         |         |
| Oleic acid               |             | 0.4   |         |         |
| Time, min.               | 2.5         | 2.5   | 2.5     | 2.5     |
| Pulp pH                  | 11.2        | 11.2  | 11.0    | 10.9    |

The results of the test follow:

| Product                    | Weight, per cent | Assay, per cent |                | Dist., per cent |                |
|----------------------------|------------------|-----------------|----------------|-----------------|----------------|
|                            |                  | $\text{SrCO}_3$ | $\text{SiO}_2$ | $\text{SrCO}_3$ | $\text{SiO}_2$ |
| Strontianite Concentrates: |                  |                 |                |                 |                |
| Rougher                    | 35.0             | 97.6            | 2.4            | 57.4            | 2.1            |
| Cleaner                    | 16.5             | 88.8            | 11.2           | 24.6            | 4.5            |
| Composite                  | 51.5             | 94.8            | 5.2            | 82.0            | 6.6            |
| Silica Rejects             | 48.5             | 22.1            | 77.9           | 18.0            | 93.4           |
| Composite Feed             | 100.0            | 50.5            | 40.5           | 100.0           | 100.0          |

*Example XI*

A mixture composed of approximately equal quantities of barite and quartz was ground to pass 65 mesh and subjected to flotation in a manner similar to that described in Example IV. The quantities of reagents, expressed in pounds per ton of flotation feed, employed for flotation of the quartz from the barite were as follows:

| Reagent                  | Conditioner |       | Rougher | Scavenger | Cleaner |       |
|--------------------------|-------------|-------|---------|-----------|---------|-------|
|                          | No. 1       | No. 2 |         |           | No. 1   | No. 2 |
| Caustic soda             | 0.7         |       |         |           | 0.4     | 0.4   |
| Sodium hexametaphosphate | 2.0         |       |         |           | 0.05    | 0.10  |
| Lead nitrate             | 1.0         |       |         |           |         |       |
| Sodium oleate            |             | 1.0   |         |           | 0.8     |       |
| Frother B-23             |             |       | 0.1     | 0.1       | 0.1     | 0.1   |
| Time, min.               | 2.5         | 2.5   | 2.5     | 4.0       | 2.5     | 2.5   |
| Pulp pH                  | 11.2        | 11.1  | 10.8    | 10.2      | 10.7    | 10.6  |

The rougher and scavenger silica froths were combined and cleaned twice by refloating in the same cell using tap water for dilution with the

reagents as indicated. The results of the test are as follows:

| Product              | Weight, per cent | Assay, per cent   |                  | Dist., per cent   |                  |
|----------------------|------------------|-------------------|------------------|-------------------|------------------|
|                      |                  | BaSO <sub>4</sub> | SiO <sub>2</sub> | BaSO <sub>4</sub> | SiO <sub>2</sub> |
| Barite Concentrates: |                  |                   |                  |                   |                  |
| Rougher.....         | 47.6             | 93.9              | 6.1              | 94.2              | 5.6              |
| Cleaner.....         | 1.9              | 65.4              | 34.6             | 2.6               | 1.2              |
| Composite.....       | 49.5             | 92.8              | 7.2              | 96.8              | 6.8              |
| Silica Rejects.....  | 50.5             | 3.0               | 97.0             | 3.2               | 93.2             |
| Composite Feed.....  | 100.0            | 47.4              | 52.6             | 100.0             | 100.0            |

*Example XII*

A sample of barite table concentrates was obtained from operating plant near Cartersville, Georgia. The table concentrates containing barite associated with iron oxides and quartz together with minor quantities of feldspar and other silicate gangue minerals were being ground and treated by flotation to reject silica and to recover an enriched barite-iron product. A head analysis of the sample gave 62.6 percent BaSO<sub>4</sub>, 29.8 percent SiO<sub>2</sub>, and 5.4 percent Fe<sub>2</sub>O<sub>3</sub>.

A 250-gram portion of the sample was wet ground in a laboratory rod mill to pass 65 mesh. The ground pulp was transferred to a mechanical flotation cell and diluted with tap water to give a pulp containing about 25 percent solids. Activation and flotation of the siliceous gangue constituents from the retarded barite and iron oxides was effected by the following quantities of reagents expressed in conventional pounds per ton of flotation feed:

| Reagent                        | Conditioner |       | Rougher | Cleaner |       |
|--------------------------------|-------------|-------|---------|---------|-------|
|                                | No. 1       | No. 2 |         | No. 1   | No. 2 |
| Caustic soda.....              | 1.0         | ----- | -----   | 0.5     | 0.4   |
| Sodium hexameta-phosphate..... | 1.5         | ----- | -----   | 0.04    | 0.04  |
| Sodium oleate.....             | -----       | 1.0   | -----   | -----   | ----- |
| Oleic acid.....                | -----       | 1.0   | 0.5     | 0.16    | ----- |
| Magnesium chloride.....        | -----       | 1.0   | -----   | -----   | ----- |
| Time, min.....                 | 2.5         | 2.5   | 5.0     | 2.5     | 2.5   |
| Pulp pH.....                   | 11.1        | 10.8  | 10.5    | 10.8    | 10.7  |

The results of the test are as follows:

| Product              | Weight, per cent | Assay, per cent   |                  |                                | Dist., per cent   |                  |                                |
|----------------------|------------------|-------------------|------------------|--------------------------------|-------------------|------------------|--------------------------------|
|                      |                  | BaSO <sub>4</sub> | SiO <sub>2</sub> | Fe <sub>2</sub> O <sub>3</sub> | BaSO <sub>4</sub> | SiO <sub>2</sub> | Fe <sub>2</sub> O <sub>3</sub> |
| Barite Concentrates: |                  |                   |                  |                                |                   |                  |                                |
| Rougher.....         | 62.3             | 83.7              | 5.6              | 7.9                            | 83.3              | 11.7             | 91.9                           |
| Cleaner.....         | 6.8              | 56.5              | 37.3             | 3.9                            | 6.1               | 8.8              | 4.9                            |
| Composite.....       | 69.1             | 81.0              | 8.7              | 7.5                            | 89.4              | 20.2             | 96.8                           |
| Silica Rejects.....  | 30.9             | 21.3              | 77.0             | 0.6                            | 10.6              | 79.8             | 3.2                            |
| Composite Feed.....  | 100.0            | 62.6              | 29.8             | 5.4                            | 100.0             | 100.0            | 100.0                          |

The beforementioned examples of practice illustrate the wide range of applicability of our method for the flotation of siliceous gangue constituents from economic nonmetallic minerals including bone phosphate of lime (tricalcium phosphate), calcite, barite, strontianite, and witherite. While we have disclosed the preferred embodiments of our invention, it will be readily apparent to those skilled in the art that many variations and modifications may be made therein without departing from the spirit of the invention.

What is claimed:

1. A process for beneficiating ores of nonmetallic minerals of the class consisting of calcite, barite, strontianite, witherite, and tricalcium phosphate containing siliceous gangue materials which comprises blunging an aqueous pulp of the comminuted ore in the presence of sufficient hydrated lime to establish a pulp pH of at least about 11, thereafter removing the lime remaining in solution, until said pulp contains not more than 100 parts per million of soluble lime, and then subjecting said pulp to agitation and aeration in the presence of a quantity of caustic alkali to establish a pulp pH at least as alkaline as pH 10, and an alkali-soluble inorganic phosphate selected from the group consisting of metaphosphates and polyphosphates, together with an anion-active collecting agent selected from the class consisting of fatty acids and resin acids and mixtures of fatty and resin acids and soaps thereof, whereby siliceous gangue is floated and beneficiated nonmetallic mineral is depressed and recovered.

2. A process for beneficiating ores of nonmetallic minerals of the class consisting of calcite, barite, strontianite, witherite, and tricalcium phosphate containing siliceous gangue materials which comprises blunging an aqueous pulp of the comminuted ore in the presence of hydrated lime to establish a pH of at least about 11, then adding thereto soda ash to precipitate the lime remaining in solution as calcium carbonate, and thereafter subjecting said pulp to agitation and aeration in the presence of an alkali-soluble inorganic phosphate selected from the group consisting of metaphosphates and polyphosphates, together with an anion-active collecting agent selected from the class consisting of fatty acids and resin acids and mixtures of fatty and resin acids and soaps thereof, whereby siliceous gangue is floated and beneficiated nonmetallic mineral is depressed and recovered.

3. The process of claim 1 wherein the alkali-soluble inorganic phosphate employed comprises sodium hexametaphosphate.

4. The process of claim 1 wherein talol is employed as the collecting agent.

5. The process of claim 1 wherein oleic acid is employed as the collecting agent.

6. The process of claim 2 wherein sodium hexametaphosphate is employed as the alkali-soluble inorganic phosphate.

7. The process of claim 2 wherein talol is employed as the collecting agent.

8. The process of claim 2 wherein oleic acid is employed as the collecting agent.

JULIUS BRUCE CLEMMER.

CARL RAMPACEK.

REFERENCES CITED

The following references are of record in the file of this patent:

UNITED STATES PATENTS

| Number    | Name                 | Date          |
|-----------|----------------------|---------------|
| 2,363,029 | Weinig               | Nov. 21, 1944 |
| 1,780,022 | Littleford           | Oct. 28, 1930 |
| 1,914,694 | Lange                | June 20, 1933 |
| 1,914,695 | Lange                | June 20, 1933 |
| 2,289,741 | Tartarton            | July 14, 1942 |
| 2,383,467 | Clemmer and Clemmons | Aug. 28, 1945 |